

July 28, 1931.

R. L. FRINK

1,816,322

METHOD OF RETAINING AND SEALING FURNACE STRUCTURES

Filed Dec. 16, 1926



Fig. 2



Fig. 1



Fig. 3.

INVENTOR.

Robert L. Frink.  
BY  
Day, Oberlin & Day  
ATTORNEYS.

## UNITED STATES PATENT OFFICE

ROBERT L. FRINK, OF LANCASTER, OHIO

## METHOD OF RETAINING AND SEALING FURNACE STRUCTURE

Application filed December 16, 1926. Serial No. 155,329.

This invention relates to method of retaining and sealing linings resistant to erosion where there is more or less chemical action and heat, and in its more specific aspects, it has reference to linings for furnaces treating materials in industrial usages such as involve severe action along heated zones of contact. For example, in glass melting tanks, the linings are subjected to very drastic conditions. Likewise with copper refining furnaces, also boiler furnaces, particularly those fired by powdered coal, etc., where the erosion is very severe. Very durable or highly refractory materials are known that offer advantages but their high cost has rendered their use prohibitive in the dimensions required in the prevalent self-supporting types of construction. Moreover, with such refractory materials as mullite, etc., the heat-conductivity is such that these materials if used alone would permit excessive heat losses through the walls. In accordance with my present invention, it now becomes possible to secure a highly-resistant surface together with the other qualities desirable at the same time, and coincidentally produce a sealing of the joints.

To the accomplishment of the foregoing and related ends, the invention, then, consists in the features hereinafter fully described and particularly pointed out in the claims, the following description and the annexed drawings illustrating but a few of the various forms in which the principle of the invention may be used.

In said annexed drawings:—

Fig. 1 is a fragmentary isometric and sectional view showing a portion of a wall and floor construction embodying the present invention; Fig. 2 is a similar view of a modification; and Fig. 3 is a sectional view illustrating the invention as applied to effect a seal between joints.

The reference numerals 1 and 2 in the drawings designate facing slabs or blocks of highly resistant or durable material. This may be selected as desirable for a particular usage in view. For example, with a glass melting furnace or tank, mullite or sillimanite may be employed. Back of the facing

slabs are support or backing blocks 3, 4, of inferior material and which may be of less density. Blocks 5 and 6 of ordinary fireclay material form the base, and a block 7 of similar material may be arranged above. By providing the blocks 6 and 7 with under-cuts or rebates or the like, as for instance at 8, and correspondingly shaping the coacting edges of the facings 1 and 2, the latter will be restrained against displacement forwardly and at the same time they are held against the backing 3 and 4. As a further safeguard, there may be provided a sort of dovetailing of more or less pronounced form, as at 10 in the mating edges of the facing slabs so as to assist in retaining these in relation. In assembling the construction as shown in Fig. 1, the floor or base blocks 5, 6, are laid in position and then the backing blocks 3, 4. The facing slabs 1 and 2 are now set in position and then the top block 7 which with its overhanging edge serves to maintain the facing in position.

In some instances, I not only secure the respective members together but also effect a seal by providing in the mating surfaces grooves which may be of circular or square cross section for instance as at 11 or 12 or of double under-cut cross section as at 2. Such grooves, with the respective blocks assembled, present then longitudinal channels involving both mating surfaces, and these channels are then filled with a locking key which may be of square section as at 13, which is preferable for certain kinds of seals.

Preferably and most conveniently, such a key may be provided by forcing in a plastic mass which when properly set will afford a suitable mechanical tie. As to the characteristics of such mass, it is desirable of course that it be capable of resisting temperatures to which the wall structure may be subjected in use, and accordingly the particular material may vary as determined by the usage in view. It is desirable also in most cases at least that the key mass have a coefficient of expansion and contraction practicably related to that of the blocks tied together or seal to be made. In the case of glass furnaces, I prefer to make up a mixture of dis-

integrated sillimanite with a binder comprising silica, boric acid, thorium or zirconium oxide, magnesium oxide and magnesium chloride, the respective quantities of each of the constituents being determined by the use to which it is to be applied, i. e., the relative co-efficient of expansion between the parts to be joined, or the conditions under which a seal is to be made and maintained; 10 in each case, the quantity of magnesium oxide and magnesium chloride to be used will depend upon the amount of cementing action desired. Just enough water is added to dampen the mass and make it adequately 15 flowable to be inserted into the channels, and these having been filled from a convenient point of access, usually at the end, the mass is allowed to dry out, and is ultimately set to final condition by heat, the temperature 20 being such that incipient fusion or softening to an extent of allowing the adherence of the particles occurs. Where a key effect only is desired, the mass should be brought to a 25 temperature above 1400° C. unless the position in which the key is used and the temperature to which it is subjected is a mere nominal temperature of from 1200° to 1300° C., where it would then be feasible to use a mixture 30 having a lower melting point, as by the addition of alkali borates or carbonates. It is advisable that the softening temperature be maintained somewhat longer in order to allow of chemical and physical adjustments in the mass. It will then be found that the 35 plastic material has become a rigid key whose fusion point is so high that it mechanically holds in the conditions of usage to which the furnace is thereafter subjected. The firing temperature for the setting of the plastic key mixture will of course vary with the particular material employed, but where such material is substantially of a sillimanite and 40 boron silicate type instanced above, a temperature of 1400° to 1500° C. or more will 45 be desirable.

As shown in Fig. 3, members may be joined with a seal to form hollow bodies or conduits, as for a recuperator system.

It has been found that to construct a recuperator tile by any of the present known methods, that produce the same in an integral piece, is unsatisfactory because of the variation of temperatures that occur, and the continued subjection of high temperatures over long periods of time causes such tiles to crack, especially where the partition member 9' is subjected to a higher temperature than the walls 9. An unequal or differential expansion occurs between the walls 9 55 and section 9' causing cracking and disintegration. It will be appreciated that when these tiles are used in recuperators either the exterior is subjected to a temperature of atmospheric air while the gases flowing through the interior may have a temperature 60

of 1200° or 1300° C., or the conditions may be vice versa.

To also meet these conditions and avoid such cracking of the tiles or conduits, with consequent leakage of the ingoing air and outgoing hot gases, thus necessitating the closing down of the furnace, my invention is found entirely satisfactory when properly executed, and while the principle and the elements embodied are substantially the same 70 whether used as a seal or a key, when used as a seal I preferably employ the following procedure:

Grooves are ground or formed into the mating surfaces between members 9 and 9'. The parts are brought into the required alignment and a mixture of sillimanite or mullite with boric acid, thoria or zirconium oxide is compounded with magnesium oxide and chloride, the mass is moistened and is then 80 injected by means of a pressure device or gun into the recesses as shown in Fig. 3 until filled, as at 13. This is preferably done during the building of the recuperator or other furnace parts. When heat is applied 85 and the masses at 13 are sintered or fused, gases are evolved and some shrinkage takes place, and to govern the quantity of shrinkage required to compensate for differential movements between members 9 and 9', I may add varying quantities of alkali, carbonates, and raw fireclay which has been deflocculated or contains the larger possible quantity of flocculant or colloidal material.

Should it be desired that the construction 90 be more or less monolithic it is then advisable to add increased quantities of alkali and carbonates to thereby lower the fusion point, creating a greater quantity of glassy substance 95 and obtain a relatively larger surface of plastic material in contact with the mating surfaces.

It will thus be seen that with a construction 100 on the general lines described, advantage may be taken of the superior resistant properties of costly and difficultly workable facing slabs in relatively thin section, and such lining may be successfully backed up or used in conjunction with cheaper and in some instances better insulating substances, the assemblage being adequately held together in use by the overhanging engagement or by the plastically-introduced key or both or seal to close 105 passages that might allow circulation of gases, as in recuperators, or fluids, as between the notch block and floater, or the bonds between spouts and base walls, etc. as circumstances may make advisable, the wedge surfaces or retreating wedge surfaces of the respective 110 members making an effective and durable interlock in engagement whether initially rigid or plastic. The extent to which the facing 115 will be applied will of course depend upon the particular usage in hand. In some cases, the entire side walls and the floor being cov-

ered, and in other cases only the side wall will require the facing. In other cases yet, all of the side wall will not require facing but only the zone at the upper part where the material being heated has its general range of exposed surface as a fluid level line contacting the wall.

Moreover, irrespective of the particular character of the members to be joined, whether in a solid wall or a hollow built-up structure, the wedging or locking member provides holding or sealing functions or both, and by the terms wedging member or locking member hereinafter, I contemplate either or both such holding and sealing functions.

Other modes of applying the principle of the invention may be employed, change being made in the details set forth, provided the means and steps stated in the following claims or the equivalent of such be employed.

I therefore particularly point out and distinctly claim as my invention:—

1. In construction of the character described, the combination of heat-resistant members having apposed surfaces provided with recesses, and a locking member fused in such recesses the locking member being glass-like in character.

2. In construction of the character described, the combination of heat-resistant members having apposed surfaces provided with recesses, and a locking member of glass-like composition fused in such recesses.

3. In construction of the character described, the combination of a facing block resistant against action of material to be treated in contact therewith, a backing of less resistant material, and heat resistant locking members for holding said facing against the backing.

4. In construction of the character described, the combination of a facing block substantially resistant against action of material to be treated in contact therewith, a backing of less resistant material, and heat resistant locking members comprising upper and lower blocks having non-planar surfaces for holding said facing against the backing.

5. In construction of the character described, the combination of a refractory facing block highly resistant against action of materials to be treated in contact therewith, a backing of less resistant material, and fusible locking members engaging the facing and backing.

6. In construction of the character described, the combination of a facing block resistant against the action of materials to be treated in contact therewith, a backing of less resistant material, upper and lower blocks having wedge surfaces for holding said facing against the backing, and intermediate locking members engaging the facing and backing and fused in place.

7. A method of making a construction of

the character described, which comprises apposing members part at least of which are refractory, and sealing such members together by applying a fusible material, and heating.

8. A method of making a construction of the character described, which comprises apposing heat-resistant members having recesses, forcing into such recesses a plastic locking material capable of setting when heated, and heating.

9. A method of making a construction of the character described, which comprises apposing heat-resistant members having mating channels, forcing a plastic locking material into such channels, and fusing at least a portion of the locking material.

10. A method of making a construction of the character described, which comprises apposing a facing and a backing having mating channels, forcing a plastic material into such channels, and subjecting the material to heat to set the same into required rigid form.

11. A method of making a construction of the character described, which comprises setting up a backing apposing a refractory facing thereagainst, said backing and facing having mating channels so formed as to contact with material therein to key the backing and the facing together, forcing into the channels a plastic material capable of setting when heated, and heating.

12. In a wall made up of a plurality of apposed members, the combination with recesses in adjacent faces of said members, of a keying and sealing member disposed in said recesses and fused to said members.

Signed by me this 14th day of December, 1926.

ROBERT L. FRINK.

105

110

115

120

125

130